

# UNITED STATES PATENT OFFICE.

CHARLES BASKERVILLE, OF NEW YORK, N. Y.

## COATING FERROUS METALS.

1,378,439.

Specification of Letters Patent.

Patented May 17, 1921.

No Drawing.

Application filed June 25, 1914. Serial No. 847,823.

To all whom it may concern:

Be it known that I, CHARLES BASKERVILLE, a citizen of the United States, residing at New York city, in the county of New York and State of New York, have invented certain new and useful Improvements in Coating Ferrous Metals, of which the following is a specification.

The present invention relates to the coating of ferrous metals under which term I include cast iron, wrought iron, and steel, the said coating being performed either with lead, or with an alloy of lead and antimony.

In the coating of ferrous metals with lead, I have found that it is preferable to coat the ferrous metal first either with antimony, either alone or in the form of an alloy containing antimony, the object of this preliminary coating being to form an article which will very readily take up a coating of metallic lead.

In the coating of metallic iron with an alloy of lead and antimony, the treatment of the ferrous metal with a preliminary layer containing antimony is not necessary, but in some instances is advisable.

It is obvious that the coating may cover either the entire surface of the article of ferrous metal, or a portion only of the surface.

Iron or steel possesses sufficient strength for use in very many connections in which its use is prohibited, since the metal, particularly in contact with water, aqueous solutions and acids, undergoes more or less oxidation, corrosion or rust.

A particular use to which iron could be put, if it were not for its tendency to rust or corrode, is the preparation of plates of filter presses, although the invention may be applied to iron or steel, either in the form of plates or sheets, or rods or wires, or the invention may be applied to the treatment of objects made of cast iron, which may or may not have been machined, and in the treatment of machined iron, the iron may be machined in places only, or over its entire surface.

I give the following examples of the carrying out of this process:—

### Example A.

Wrought iron or steel is first pickled in acids in substantially the usual manner; it

may then be washed and dipped into a molten alloy of lead and antimony (3 to 13% of the latter) and thereafter dipped into molten lead. As the metal thus coated emerges from the last bath of molten metal it may be first quenched in oil and then either in water or a soap solution, or if desired the quenching in oil may be omitted.

In the pickling of certain varieties of iron, particularly cast iron, hydrofluoric acid may be used in the pickling bath as has been already proposed either as an aqueous solution of this acid alone, or an aqueous solution of this acid mixed with other acids, with or without salts.

In this process a suitable flux, which may or may not contain zinc chlorid, may be placed upon the molten lead-antimony alloy, or the molten lead, or both, in order to cause the lead or alloy to more readily attach itself to the iron.

This process is applicable, to sheets, rods or wires, or other iron or steel articles.

### Example B.

Wrought iron or steel is first pickled in acids, may then be washed if desired, and is then dipped into a molten alloy of lead and either antimony or zinc, or an alloy containing lead, antimony and zinc, which alloy has previously been subjected to the action of a low voltage high amperage, alternating electric current in the manner described in any one or more of the U. S. patents to Goodson Nos. 900,846, 900,847, 987,448 and 1,061,066, and Reissue 12,779.

The article may then be dipped or immersed into a bath of molten lead, which bath may or may not have previously been treated electrically, as above referred to, or if desired, this second dipping may be into a bath composed of an alloy of different composition from that used in the first step, which alloy may or may not have been treated electrically by the means above referred to. The use of a flux, floating upon the bath of molten alloy or metal, which flux may or may not contain zinc chlorid, is optional. The metal article under treatment, as it emerges from the last bath of molten metal or alloy, may optionally be quenched in oil, water, soap solution, or mixtures or sequences of these. If it is desired to coat cast iron according to this

process the process of pickling may involve the use of hydrofluoric acid as above referred to.

*Example C.*

5 Cast iron is first cleaned or pickled, in a bath of dilute hydrofluoric acid, which may for example be of 2-20%. The iron is then washed, is then subjected to the action of 10 suitable flux, then treated with a bath of lead and antimony (from 3 to 13% of the latter) which alloy may or may not have been treated electrically as above referred to.

15 As an optional method of coating the cast iron with the antimony, the cast iron may be dipped and allowed to stand for a short time, in a solution of antimony chlorid ( $SbCl_3$ ) and subsequently washed or swilled.

20 The iron coated with either antimony or an antimony lead alloy, is placed in a mold, in such a manner that the plated iron forms a core around which molten lead, or an alloy of lead is poured, and the material allowed to cool sufficiently for the lead or alloy to 25 solidify. The lead or alloy of lead used in this casting step may or may not have been subjected to the electrical treatment above referred to.

30 *Example D.*

The iron may be pickled, either by the well known methods, or by the method involving the use of hydrofluoric acid, and may then receive a thin coating of antimony, 35 either by treatment with a solution of antimony chlorid or by immersion in a bath of molten alloy of lead and antimony, and the coated metal is then dipped or immersed in the bath of coating metal.

40 The preliminary coating of antimony may be produced in a variety of ways, for example those above referred to, or the iron, which may have been pickled, if desired, is dipped into a solution of hydrosulfite (for 45 example the technical products sold as "hydrosulfite," which contains  $Na_2S_2O_4$ , as its principal ingredient, but which ordinarily is not pure), after which the iron may be dipped or immersed in a solution of antimony chlorid. The coating with antimony may 50 also be produced by dipping or immersing clean iron, in an acid solution of antimony chlorid (a solution of  $SbCl_3$  so-called "butter of antimony," containing free HCl) and 55 allowing the antimony to deposit on the surface of the iron. Another method of coating the iron with antimony, is to subject the iron article, having a comparatively clean surface, to the vapors of metallic antimony, 60 formed by subjecting metallic antimony to an elevated temperature, or by distilling a mixture of antimony oxid and a carbonaceous material. Another method is by electroplating clean iron, with a thin coating of

antimony. Another method consists in 65 sherardizing the iron articles with antimony.

As specific example of this mode of treatment the following are given:

- D1. a. Pickle iron in  $H_2SO_4$ , 70  
 b. Wash in water  
 c. Let stand in antimony trichlorid solution, until a coating of antimony has formed on the iron, such solution may consist of: 75  
     40 oz.  $H_2O$   
     10 oz. HCl  
     1 oz.  $SbCl_3$  solution (so-called "butter of antimony")  
 d. Wash in water 80  
 e. Dip in cut zinc flux,  
 f. Dip in molten lead.  
 D2. a. Pickle the iron in  $H_2SO_4$ ,  
 b. Wash in water  
 c. Dip in hydrosulfite solution, 85  
 d. Dip in antimony trichlorid solution (described above) until deposit forms,  
 e. Wash in water,  
 f. Dip in cut zinc flux, 90  
 g. Dip in lead.  
 D3. a. Pickle iron in  $H_2SO_4$ ,  
 b. Wash in water  
 c. Immerse in solution of  $SbCl_3$ , 95  
     40 oz.  $H_2O$   
     10 oz. HCl  
     1 oz. soln.  $SbCl_3$   
 d. Dip in molten metal, (lead or lead-antimony alloy)  
 D4. a. Pickle iron in  $H_2SO_4$ , 100  
 b. Wash in water,  
 c. Immerse in solution of  $SbCl_3$  +  $ZnCl_2$ ,  
     40 oz.  $H_2O$   
     10 oz. HCl 105  
     1 oz. soln.  $SbCl_3$ ,  
     8 oz. approx.  $ZnCl_2$   
 d. Dip in molten metal (lead or lead-antimony alloy).

The metal coated with antimony according to either of the methods described under D1, D2, D3 or D4, may then be placed in a mold, in such a manner as to form the core of the mold, and molten lead or other molten metal may be cast around the coated iron or steel, in order to form a coating of any desired thickness, which coating will closely adhere to the metal base, or the iron coated with antimony may be dipped into a bath of molten lead or alloys of lead, such as above stated.

The coated articles, in any of these examples may be quenched in oil or water or soap solution, as above described.

Attempts have heretofore been made, and 125 various patents have been secured for processes of coating iron with lead, but in producing a strong and close union of the iron

or steel, with the lead, it has been necessary to carefully manipulate the lead and iron. I have found that by my method, which involves the application of a layer of antimony, or an alloy containing antimony to the iron, it is a very simple matter to afterward apply metallic lead in such a manner as to produce a complete union between the lead and the iron.

10 What I claim is:—

1. A method of coating ferrous metals which comprises coating said metals first with metallic antimony in a substantially pure condition, and thereafter coating with a material containing metallic lead.

2. A method of coating iron or steel, which comprises treating the same, with a solution containing an antimony compound, and thereafter coating with a material containing metallic lead.

3. A method of coating a ferrous metal which comprises pickling the same in a bath containing hydrofluoric acid, treating with a solution of an antimony salt, thereafter immersing in a bath containing molten lead, said bath carrying on its surface, a flux containing zinc chlorid, and thereafter quenching the coated metal in a suitable liquid.

4. A process of coating ferrous articles which comprises (a) pickling in acid, (b) treating with a solution containing a hydro-sulfite, (c) treating with a solution of an antimony compound, and thereafter dipping into a molten lead-containing bath.

35 5. In the coating of iron, steps of pickling the iron, thereafter immersing at least a portion of the article in a bath containing  $\text{Na}_2\text{S}_2\text{O}_4$ , and thereafter coating the same

with a preliminary coating containing antimony.

6. A ferrous metal having a coating of metallic lead, said coating being united to said ferrous metal by a layer of an alloy consisting of antimony and lead.

7. A method of coating a ferrous metal article which comprises pickling the same in a bath containing hydrofluoric acid, dipping the same into a solution containing a hydro-sulfite, subjecting said article to the action of an acid solution of an antimony salt, and thereafter coating the same with a material containing lead, and thereafter quenching the coated article in a suitable liquid.

8. A process of coating ferrous articles which comprises (a) pickling in acid, (b) treating with a solution containing a hydro-sulfite, (c) treating with a solution of an antimony compound, (d) treating with a zinciferous fluxing agent, and thereafter dipping into a molten lead-containing bath.

9. A process of uniting a coating layer of a lead-containing metallic substance to a ferrous metal base which comprises subjecting a ferrous article to the action of a solution of an antimony compound whereby antimony is coated thereupon, and thereafter subjecting the ferrous article with such coating thereupon to the action of a bath of the said lead-containing metallic substance.

In testimony whereof I affix my signature in presence of two witnesses.

CHARLES BASKERVILLE.

Witnesses:

THOMAS F. O'KEEFFE,  
JOSEPH A. MAGUIRE.